

# UNITED STATES PATENT OFFICE.

HEINRICH GRÜNWALD, OF GRIESBORN, NEAR BOUS-ON-THE-SAAR, GERMANY.

## PAINT FOR PROTECTING METALS FROM RUSTING.

1,179,176.

Specification of Letters Patent. Patented Apr. 11, 1916.

No Drawing.

Application filed August 4, 1914. Serial No. 855,063.

*To all whom it may concern:*

Be it known that I, HEINRICH GRÜNWALD, a subject of the King of Bavaria, residing at No. 218 Griesborn, near Bous-on-the-Saar, 5 Germany, have invented a certain new and useful Paint for Protecting Metals from Rusting; and I do hereby declare the following to be a full, clear, and exact description of the invention.

10 The present invention relates to the art of rust proofing metals and consists in the preparation of an improved rust proofing composition.

The fact that oils, such as linseed oil, 15 rape-seed oil, etc., when combined at suitable temperatures with sulfur, yield certain products of condensation, is well known. Chlorid of sulfur serves equally as well as sulfur and the term "sulfur" is used herein- 20 after and in the claims in a sense broad enough to include such a compound. Also other oils, vegetable as well as animal ones yield on treatment with sulfur or chlorid of sulfur at suitable temperatures, similar 25 products of condensation. Depending upon the proportions of the reagents entering into the mixture and upon the temperature at which the reaction is carried out, products are obtained which vary all the way from 30 syrupy consistency to brittle masses.

Products of a tough, rubber-like character may be obtained, if an oil such as linseed oil, or a mixture of the same with resin, is heated to a temperature from 170° C. to 35 200° C. and while at this temperature sulfur is added little by little until the mixture is of such consistency that it can be drawn out into threads that do not readily break. On cooling, this product discloses physical 40 properties closely approaching those of rubber.

Through extended researches which have resulted in the present discovery, it has been found that these masses or mixtures 45 of the same with asphalt, pitch tar or other substances which are useful for rust proofing metals, when applied in suitable manner to metal surfaces, adhere extremely firmly thereto, stretch with the same without crack- 50 ing when the metal expands or contracts by

reason of temperature change, protect the metal against moisture, insulate it against the action of electric currents and forms an efficient protection against erosion and like 55 mechanical wear upon the surface.

The following example serves to illustrate the invention: One hundred (100) parts by weight of linseed oil is mixed with one hundred parts (100) by weight of American resin, during agitation and in the presence 60 of heat. When the temperature of the mixture has reached from 170° C. to 200° C., small portions of sulfur are added gradually until a sample taken from the mass, draws 65 out to a thread. When this condition has been attained,—the temperature being such that it may serve to melt the added ingredients,—one hundred (100) parts tar oil are added or some other solvent such as a low 70 boiling fraction of raw petroleum, carbon tetrachlorid, carbon bisulfid, benzol, etc. To this are added five hundred (500) parts of coke oven tar (free from water) and the metal objects, such as iron pipes, then 75 dipped therein. Upon cooling, the objects 80 are found to be covered with an extremely adherent protective coating possessing the characteristics above mentioned. It is possible furthermore to dissolve the above described sulfur-oil-resin mixture after it has 85 cooled to 100° C., in varnish or in one of the other abovementioned thin fluid solvents and add thereto a solution of one hundred (100) parts asphalt in one hundred (100) parts varnish. This preparation may be 90 applied cold to the metal, and upon the evaporation of the solvent leaves a protective covering having the same characteristics as that first described.

I claim:

1. A paint for protecting metals from rusting, comprising a solution of the condensation products of oil, resin and sulfur, which condensation products are capable, at a suitable temperature, of being drawn out 95 to threads, such solution being intimately intermixed with a tarry liquid.

2. A paint for protecting metals from rusting, comprising a solution of the condensation products of oil, resin and sulfur, 100

which condensation products are capable, at a suitable temperature, of being drawn out to threads, such solution being intimately intermixed with a tarry liquid consisting of 5 a solution of asphalt in an equal part of varnish.

In testimony whereof I have signed my

name to this specification in the presence of two subscribing witnesses.

HEINRICH GRÜNWALD.

Witnesses:

FRITZ MOLIBOR,  
CARL DRAPPER.